# EUROPEAN PATENT SPECIFICATION

(11) **EP 2 171 131 B1**
(45) Date of publication and mention of the grant of the patent: **29.12.2010**
(21) Application number: 08786597.8
(22) Date of filing: 30.07.2008
(51) Int. Cl.: C25D 3/66, C25D 3/02, C25F 3/16

(54) **METHOD TO ELECTRODEPOSIT METALS USING IONIC LIQUIDS IN THE PRESENCE OF AN ADDITIVE**
VERFAHREN ZUR ELEKTRODEPONIERUNG VON METALLEN MITHILFE IONISCHER FLÜSSIGKEITEN UNTER VERWENDUNG EINES ZUSATZSTOFFS
PROCEDE POUR ELECTRODEPOSER DES METAUX A L'AIDE DE LIQUIDES IONIQUES EN PRESENCE D'UN ADDITIF

(30) Priority: 02.08.2007 EP 07113717; 07.08.2007 US 954434 P
(43) Date of publication of application: 07.04.2010
(73) Proprietor: Akzo Nobel N.V., 6824 BM Arnhem (NL)
(72) Inventor: KUZMANOVIC, Boris, NL-3521 DB Utrecht (NL); NABUURS-WILLEMS, Lamberdine, Johanna, Willemina, M, NL-5825 HT Overloon (NL); VAN STRIEN, Cornelis, Johannes, Govardus, NL-6662 HH Elst (NL); WELTER, Franz, Winfried, 52379 Langerwehe (DE); SPEELMAN, Johanna, Christina, NL-7231 BP Warsveld (NL)
(74) Representative: Schalkwijk, Pieter Cornelis
(86) International application number: PCT/EP2008/059962
(87) International publication number: WO 2009/016189

(56) References cited:
- US-A1- 2004 061 919
- US-A1- 2004 150 866
- WANG P ET AL: "GELATION OF IONIC LIQUID-BASED ELECTROLYTES WITH SILICA NANOPARTICLES FOR QUASI-SOLID-STATE DYE-SENSITIZED SOLAR CELLS" JOURNAL OF THE AMERICAN CHEMICAL SOCIETY, AMERICAN CHEMICAL SOCIETY, WASHINGTON, DC, US, vol. 125, no. 5, 2003, pages 1166-1167, XP001172435 ISSN: 0002-7863

## Description

The present invention relates to a method to electrodeposit a metal on a substrate using an ionic liquid as the electrolyte in the presence of an additive, and to the use of said additive to increase the layer thickness of the deposited metal layer.

An ionic liquid is a salt in which the ions are poorly coordinated, which results in these solvents being liquid at temperatures below 100°C. Many are liquid even at room temperature. At least one ion in an ionic liquid has a delocalized charge and one component is organic, which prevents the formation of a stable crystal lattice. Ionic liquids generally have very low vapour pressure and thus, in contrast to many conventional solvents, produce virtually no hazardous vapours. It is known that, in general, ionic liquids may be used in many applications, e.g. as reaction solvents, extraction solvents, electrolytes in batteries and electrodeposition, catalysts, heat exchange fluids, as additives in coatings.

Well-known systems include those formed from alkylpyridinium halides or dialkylimidazolium halides with an aluminium halide, and those based on choline chloride and a (hydrated) metal salt such as chromium(III) chloride. These systems have been utilized as electrolytes in electroplating, as described for example in EP 0 404 188 and EP 1 322 591.

Further, WO 2002/026381 discloses ionic liquids (eutectic mixtures) of choline chloride and a (hydrated) metal salt such as chromium(III) chloride and the use thereof in electrodeposition and electropolishing. The mixtures consist of choline chloride and the (hydrated) metal salt in a ratio of ammonium to metal ion of between 1:1 and 1:2.5 and are specifically said to be suitable for depositing chromium, cobalt, zinc or silver on a metal substrate.

Moreover, PCT/EP/2007/051329 describes a method to electroplate or electropolish a metal on a substrate wherein an ionic liquid selected from the group of
N⁺R₁R₂R₃R₄ X⁻ or
N⁺R₅R₆R₇R₈ Y⁻
is employed as electrolyte, and a metal salt added to the ionic liquid is employed as the metal source or a metal anode is used as the metal source, wherein any one of R₁ to R₈ independently represents a hydrogen, alkyl, cycloalkyl, aryl, or aralkyl group that may be substituted with a group selected from OH, Cl, Br, F, I, phenyl, NH₂, CN, NO₂, COOR₉, CHO, COR₉, or OR₉, at least one of R₅ to R₈ is a fatty alkyl chain, and one or more of R₅ to R₈ can be a (poly)oxyalkylene group wherein the alkylene is a C₁ to C₄ alkylene and the total number of oxyalkylene units can be from 1 to 50 oxyalkylene units, and at least one of R₁ to R₈ is a C₁ to C₄ alkyl chain, R₉ is an alkyl or cycloalkyl group, X⁻ is an anion having an N-acyl sulphonylimide anion (-CO-N⁻-SO₂-) functionality, Y⁻ is an anion compatible with the N⁺R₅R₆R₇R₈ ammonium cation, such as a halogenide anion, a carboxylate anion, a sulphate (both organic and inorganic sulphate), sulphonate, carbonate, nitrate, nitrite, thiocyanate, hydroxide, or sulphonylimide anion.

The use of ionic liquids as electrolytes in electrodeposition processes has several advantages. Conventional chromic acid plating processes, for example, are extremely hazardous because they mainly rely on hexavalent chromium, which is highly toxic and carcinogenic. Ionic liquids, on the other hand, may eliminate the necessity to use hexavalent chromium and allow the use of trivalent chromium, which is considered to be far less dangerous. Also, conventional chromium plating baths require the use of strong acids, which poses significant disposal problems, while the use of ionic liquids generally enables such disposal difficulties to be minimized or even eliminated. Moreover, ionic liquids are non-volatile, so they do not cause atmospheric pollution. However, a drawback to the prior art electrodeposition processes wherein an ionic liquid is used as the electrolyte is that depositing metal layers of some metals thicker than 150-200 nm is difficult or even impossible.

For some applications, such as decorative plating, having thin metal layers is acceptable. However, for applications where the metal layer needs to provide protection against wear or abrasion, or to improve hardness (functional plating), metal layers much thicker than 200 nm are required. More particularly, layers of several micrometers or even several tens of micrometers are desirable.

Hence, there is a need for improved ionic liquid-based electrodeposition systems with which metal layers of increased thickness are deposited.

Surprisingly, it has been found that by adding a particular additive to the ionic liquid-based plating baths, thicker metal layers are deposited. In more detail, the present invention relates to the use of amorphous silica, graphite powder, or a mixture thereof as additive in a process to electroplate or electropolish a metal on a substrate wherein an ionic liquid is employed as the electrolyte to increase metal layer thickness. Additionally, the invention relates to a method according to claim 7.

Additives have been added to the ionic liquid comprising electrolyte for several reasons. US 7,196,221, for example, discloses the use of brightening agents to improve the appearance of the coatings obtained in ionic liquid solvents/- electrolytes during metal plating and electropolishing processes, and in particular in chromium plating processes. The brightening agents include thiourea, saccharin, vanillin, allyl urea, nicotinic acid, citric acid, gelatin, 2-mercaptobenzothiazole, tetraethylammonium fluoride dihydrate or tetramethylammonium hydroxide pentahydrate. However, these additives have an adverse effect on the homogeneity of the deposited layer, or no effect at all.

WO 2006/074523 relates to a process for the recovery of platinum group metal, which comprises electrodeposition of the platinum group metal from an ionic liquid wherein redox reagents, complexing agents, conductivity enhancers may be present.

US 6,552,843, which is concerned with devices, such as adjustable mirrors, smart windows, optical attenuators, and displays, for controlling the reflectance and/or transmission of electromagnetic radiation, discloses a reversible electrodeposition optical modulation device employing an ionic liquid electrolyte. The ionic liquid electrolyte is comprised of a mixture of an ionic organic compound and the salt of an electrodepositable metal. The ionic organic compound comprises a heterocyclic cation such as N-alkylpyrrolidinium, pyrrolidinium, 1-alkyl-3-methylimidazolium, N-alkylpyridinium, 2-alkyl-1-pyrrolinium, 1-alkylimidazolium. The electrodepositable metal is silver, copper, tin, zinc, palladium, bismuth, cadmium, mercury, indium, lead, antimony, thallium, and alloys thereof. It is mentioned that said ionic liquid electrolyte may be rendered more viscous, semi-solid or solid by addition of organic or inorganic gelling agents. Inorganic or organic materials, including suspended carbon and dissolved dyes, may be added to the electrolyte to impart a desired colour or to reduce background reflection.

None of these documents teaches how to obtain thicker metal layers in electrodeposition processes with ionic liquid comprising electrolytes.

The term electrodeposition in this application should be understood to include both electroplating and electropolishing. By electroplating is meant the process of using electrical current to coat an electrically conductive object with a layer of metal. The preferred result is a thin, smooth, even coat of metal on the object. The primary application of electroplating is to deposit a layer of a metal having some desired property (e.g., abrasion and wear resistance, corrosion protection, lubricity, improvement of aesthetic qualities, etc.) onto a surface lacking that property. Another application uses electroplating to build up thickness on undersized parts. By electropolishing is meant smoothing and enhancing the appearance of an originally rough or uneven metal surface by coating it with a relatively thin metal layer.

The additive used according to the present invention to increase the thickness of the deposited metal layer is amorphous silica, graphite powder, or a mixture thereof.

The term amorphous silica is meant to include colloidal silica particles in any form, where the colloidal silica particles, which are also referred to as silica sols, may be derived from e.g. precipitated silica, silica gels, pyrogenic silica (fumed silica), micro silica (silica fume) or mixtures thereof. Colloidal silica according to the present invention may be modified and can contain other elements such as amines, aluminium and/or boron, which can be present in the particles and/or the continuous phase.

The colloidal silica particles can be dispersed in a substantially aqueous solvent, suitably in the presence of stabilizing cations such as K⁺, Na⁺, Li⁺, NH₄⁺, organic cations, primary, secondary, tertiary, and quaternary amines, and mixtures thereof, so as to form an aqueous silica sol. However, also dispersions comprising organic solvents, e.g. lower alcohols, acetone or mixtures thereof, also denoted as organo-silica sols, may be used. Preferably, the silica content in the sol is from about 5 to about 80% by weight.

Aqueous silica sols suitable for use according to the present invention are e.g. commercially available from Akzo Nobel. Suitable organo-silica sols are e.g. commercially available from Nissan Chemical Industries.

By graphite powder is meant finely divided carbon powder or carbon black, e.g. commercially available from Degussa.

The additive is preferably used in a quantity of at least 0.01 wt%, more preferably of at least 0.05 wt%, and most preferably of at least 0.1 wt%, based on the total weight of the electrolyte. Preferably, no more than 5 wt%, more preferably no more than 3 wt%, and most preferably no more than 1 wt% of additive is used, based on the total weight of the electrolyte. It is noted that the term electrolyte stands for the total electrolyte mixture, i.e. including dissolved metal salts and additives.

With the present invention, *i*.*e*. with the addition of the described additive(s), the layer thickness can be increased at least 10 times, more preferably at least 20 times, and most preferably at least 40 times, when compared to electrodeposition without said additive(s).

The ionic liquid employed as electrolyte is preferably selected from the group consisting of N⁺R₁R₂R₃R₄ X⁻, N⁺R₅R₆R₇R₈ Y⁻, and mixtures thereof, wherein any one of R₁ to R₈ independently represents a hydrogen, alkyl, cycloalkyl, aryl, or aralkyl group that may be substituted with a group selected from OH, Cl, Br, F, I, phenyl, NH₂, CN, NO₂, COOR₉, CHO, COR₉, or OR₉, wherein at least one of R₁ to R₄ is an, optionally branched, fatty alkyl chain, wherein R₂ can be a (C₂-C₆ alkyl)-N⁺R₁₆R₁₇R₁₈ group with R₁₆, R₁₇, R₁₈ being similar to R₁, R₃, R₄, respectively, or a C₁ to C₄ alkyl chain, and wherein one or more of R₁ to R₈ can be a (poly)oxyalkylene group wherein the alkylene is a C₁ to C₄ alkylene and the total number of oxyalkylene units can be from 1 to 50 oxyalkylene units, and wherein at least one of R₁ to R₈ is a C₁ to C₄ alkyl chain, wherein R₉ is an alkyl or cycloalkyl group, wherein X⁻ is an anion compatible with the N⁺R₁R₂R₃R₄ ammonium cation, such as a halogenide anion, a carboxylate anion, a sulphate (both organic and inorganic sulphate), sulphonate, carbonate, nitrate, nitrite, thiocyanate, hydroxide, saccharinate anion, or sulphonylimide anion, and wherein Y⁻ is an anion having a sulfonylimide anion or an N-acyl sulphonylimide anion (-CO-N⁻-SO₂-) functionality.

In one embodiment, X- is selected from the group of F⁻, Cl⁻, Br⁻, I⁻; the group of R₁₀COO⁻ anions wherein R₁₀ may be hydrogen, a C₁-C₂₂ alkyl, alkenyl or aromatic group; the group of R₁₁SO₄⁻ anions wherein R₁₁ may be absent, in which case the cation is divalent, hydrogen, a C₁-C₂₂ alkyl, alkenyl or aromatic group; the group of R₁₂SO₃⁻ anions wherein R₁₂ may be absent, in which case the cation is divalent, hydrogen, a C₁-C₂₂ alkyl, alkenyl or aromatic group; the group of R₁₃CO₃⁻ anions wherein R₁₃ may be absent, in which case the cation is divalent, hydrogen, a C₁-C₂₂ alkyl, alkenyl or aromatic group; and the group of R₁₄-N⁻-SO₂-R₁₅ anions wherein R₁₄ and/or R₁₅ independently may be hydrogen, a C₁-C₂₂ alkyl, alkenyl or aromatic group, and R₁₄ may be linked to the nitrogen atom with a carbonyl group.

A fatty alkyl chain is meant to include saturated and/or unsaturated chains and contains 8 to 22 carbon atoms; preferably, it contains 10 to 22 carbon atoms, most preferably 12 to 20 carbon atoms.

In another embodiment, an ionic liquid of the formula N⁺R₁R₂R₃R₄ X⁻ is used with R₁, R₃, and R₄ being as mentioned above and with R₂ being a (C₂-C₆alkyl)-N⁺R₁₆R₁₇R₁₈ group. Preferably, R₁₆, R₁₇, and R₁₈ are identical to R₁, R₂ and R₄, respectively, with at least one of them being an, optionally branched, fatty alkyl chain, resulting in a gemini-type structure (i.e. a symmetrical diquaternary ammonium compound).

In another embodiment, Y⁻ is based on a compound known as a sweetener. In another embodiment, N⁺R₅R₆R₇R₈ is an amine wherein the groups R₅ to R₈ are hydrogen or an alkyl or cycloalkyl, optionally substituted with OH or Cl; more preferably, at least three thereof are an alkyl, more preferably a C₁ to C₄ alkyl.

In a preferred embodiment, the ionic liquid is selected from any one of choline saccharinate, choline acesulphamate, hexadecyltrimethyl ammonium chloride, octadecyltrimethyl ammonium chloride, cocotrimethyl ammonium chloride, tallowtrimethyl ammonium chloride, hydrogenated tallowtrimethyl ammonium chloride, hydrogenated palmtrimethyl ammonium chloride, oleyltrimethyl ammonium chloride, soyatrimethyl ammonium chloride, cocobenzyldimethyl ammonium chloride, C12-16-alkylbenzyldimethyl ammonium chloride, hydrogenated tallowbenzyldimethyl ammonium chloride, dioctyldimethyl ammonium chloride, didecyldimethyl ammonium chloride, dicocodimethyl ammonium nitrite, dicocodimethyl ammonium chloride, di(hydrogenated tallow)dimethyl ammonium chloride, di(hydrogenated tallow)benzylmethyl ammonium chloride, ditallowdimethyl ammonium chloride, dioctadecyldimethyl ammonium chloride, hydrogenated tallow(2-ethylhexyl)dimethyl ammonium chloride, hydrogenated tallow(2-ethylhexyl)dimethyl ammonium methylsulphate, trihexadecylmethyl ammonium chloride, octadecylmethylbis(2-hydroxyethyl) ammonium chloride, cocobis(2-hydroxyethyl)methyl ammonium nitrate, cocobis(2-hydroxyethyl)methyl ammonium chloride, cocobis(2-hydroxyethyl)benzyl ammonium chloride, oleylbis(2-hydroxyethyl)methyl ammonium chloride, coco[polyoxyethylene(15)]methyl ammonium chloride, coco[polyoxyethylene(15)]methyl ammonium methylsulphate, coco[polyoxyethylene(17)]methyl ammonium chloride, octadecyl-[polyoxyethylene(15)]methyl ammonium chloride, hydrogenated tallow[polyoxyethylene(15)]methyl ammonium chloride, tris(2-hydroxyethyl)tallow ammonium acetate, tallow-1,3-propane pentamethyl diammonium dichloride.

Many of the above-indicated ionic liquids suitable for use according to the present invention can be prepared by a simple reaction of salts, for example by a metathesis reaction of choline chloride and sodium saccharinate (acesulphamate) to form a choline saccharinate (acesulphamate) ionic liquid, or by quaternization of the corresponding amines.

The molar ratio of the ammonium cation of the ionic liquid to the metal cation of the metal salt, which comes from the dissolved salt or from the metal anode, is preferably between 1,000:1 and 3:1. More preferred is a molar ratio of the ammonium cation of the ionic liquid to the metal cation of the metal salt of between 500:1 and 5:1, most preferred is a molar ratio between 100:1 and 7:1, this providing a good-quality metal layer, excellent dissolution of the metal in the ionic liquid, and a good balance between the cost of the process and the appearance of the plated substrate product.

Preferably, one of the metals chromium, aluminium, titanium, zinc or copper, or an alloy thereof is deposited. More preferably, chromium or aluminium is deposited, most preferably chromium. This metal deposition can be done from a metal salt dissolved in the electrolyte, for example a metal halide, preferably, but not limited to, a metal chloride. It can also be performed using a pure metal which is applied as anode (i.e. a chromium, aluminium, titanium, zinc, or copper anode). In the embodiment where a metal anode is used, the anode may be in the form of metal pieces, chunks, chips or any other suitable form known to the skilled person.

The substrate which can be electroplated or electropolished according to the present invention can be any conductive object. Preferably, it is an object which is solid metal, such as a carbon steel object, or it comprises conductive elements such as a composite material object.

The present invention furthermore relates to a method to electroplate or electropolish a metal on a metal substrate wherein an ionic liquid ionic liquid is selected from the group consisting of N⁺R₁R₂R₃R₄ X⁻, N⁺R₅R₆R₇R₈ Y⁻, and mixtures thereof, wherein any one of R₁ to R₈ independently represents a hydrogen, alkyl, cycloalkyl, aryl, or aralkyl group that may be substituted with a group selected from OH, Cl, Br, F, I, phenyl, NH₂, CN, NO₂, COOR₉, CHO, COR₉, or OR₉, wherein at least one of R₁ to R₄ is an, optionally branched, fatty alkyl chain, wherein R₂ can be a (C₂-C₆ alkyl)-N⁺R₁₆R₁₇R₁₈ group with R₁₆, R₁₇, R₁₈ being similar to R₁, R₃, R₄, respectively, or a C₁ to C₄ alkyl chain, and wherein one or more of R₁ to R₈ can be a (poly)oxyalkylene group wherein the alkylene is a C₁ to C₄ alkylene and the total number of oxyalkylene units can be from 1 to 50 oxyalkylene units, and wherein at least one of R₁ to R₈ is a C₁ to C₄ alkyl chain, wherein R₉ is an alkyl or cycloalkyl group, wherein X⁻ is an anion compatible with the N⁺R₁R₂R₃R₄ ammonium cation, such as a halogenide anion, a carboxylate anion, a sulphate (both organic and inorganic sulphate), sulphonate, carbonate, nitrate, nitrite, thiocyanate, hydroxide, saccharinate anion, or sulphonylimide anion, and wherein Y⁻ is an anion having a sulfonylimide anion or an N-acyl sulphonylimide anion (-CO-N⁻-SO₂-) functionality,
wherein a metal salt added to said ionic liquid or a metal anode is employed as metal source, and
wherein said ionic liquid comprises at least 0.01 wt%, based on the total weight of electrolyte, of an additive selected from the group consisting of amorphous silica, graphite powder, and of a mixture thereof.

The additive is preferably used in the quantities as described above.

The electrodeposition is preferably performed at temperatures below 90°C and more preferably at room temperature, in open electrodeposition vessels, but electrodeposition is not limited to these conditions.

The process according to the present invention is further illustrated by the following examples.

### EXAMPLES

### Comparative Example 1 - Electroplating of chromium from CrCl₃ hexahydrate salt onto carbon steel in cocoalkylmethyl [polyoxyethylene(15)] ammonium chloride with no additives

Chromium (III) chloride hexahydrate salt was added to cocoalkylmethyl [polyoxyethylene(15)] ammonium chloride ionic liquid containing 0.2 wt% of water and the mixture was agitated at a temperature of about 50°C until the solid salt dissolved. In the prepared solution the concentration of chromium (III) chloride hexahydrate was 75 g/kg.

About 250 ml of that solution was poured into the Hull cell equipped with an electrical heating element which had a length of 65 mm on the anode side and 102 mm on the cathode side, a 48 mm shortest anode-cathode distance, a 127 mm longest anode-cathode distance, and a depth of 65 mm. The cell was heated and the temperature was maintained at about 80°C. The liquid was agitated using a centrally positioned top-entering impeller.

Platinized titanium plate was applied as the anode and connected to the positive terminal of a DC power source, whereas carbon steel plate was used as the cathode (substrate) and connected to the negative terminal. Prior to introduction into the bath, the substrate plate was cleaned with a commercial scouring powder, washed in demineralized water, in acetone and after that in ethanol, and finally in a 4 M-HCl aqueous solution. When both plates were connected and introduced into the cell, the voltage difference was set to 30 V. The current flow was monitored on a meter connected in series.

After several hours of electroplating, the cathode was disconnected from the power source and taken out of the cell. The plate was washed in water and acetone and then dried. Chemical analysis by scanning electron microscopy combined with X-ray dispersion (SEM/EDX) of the substrate was performed. It confirmed deposition of chromium onto the carbon steel. The deposited layer thickness was measured using a thickness measurement device obtained from Fischer, Germany. The thickness was found to be lower than 0.5 µm.

### Example 2 - Electroplating of chromium from CrCl₃ hexahydrate salt onto carbon steel in cocoalkylmethyl [polyoxyethylene(15)] ammonium chloride with addition of 0.2 wt% amorphous silica

To the prepared solution of chromium (III) chloride hexahydrate salt in cocoalkylmethyl [polyoxyethylene(15)] ammonium chloride ionic liquid as described in Example 1 was added an amorphous silica aqueous colloidal solution which contained 8 wt% of active compound. The concentration of the amorphous silica in the prepared solution, expressed as the quantity of the active compound, was 1.6 g/kg.

About 250 ml of that solution was poured into the Hull cell described in Example 1. The cell was heated to a temperature of about 80°C.

The same pretreatment of the carbon steel substrate (cathode) as in Example 1 was performed, and again platinized titanium plate was applied as the anode. The potential difference was set to 30 V. The liquid was agitated using a centrally positioned top-entering impeller. The current flow between the electrodes was monitored on a meter connected in series.

After several hours of submission to the current, the cathode was disconnected from the power source and taken out of the cell. The plate was washed in water and acetone and then dried. Chemical analysis by scanning electron microscopy combined with X-ray dispersion (SEM/EDX) of the substrate confirmed deposition of chromium onto the carbon steel plate. The deposited layer thickness, measured using a thickness measurement device (Fischer, Germany), was found to be as high as 8 µm in certain regions of the substrate, which was significantly thicker than when no additive was used. As is typical for the Hull cell experiments, the layer thickness varied with the position on the substrate - in this case from 1 µm to 8 µm. To confirm these measurements a cross-cut metallographic analysis was also done. The sample of the substrate was embedded in epoxy resin and the deposit was evaluated under the microscope. The layer thickness determined in this way was in agreement with the thickness measurement device results.

### Example 3 - Electroplating of chromium from CrCl₃ hexahydrate salt onto carbon steel in cocoalkylmethyl [polyoxyethylene(15)] ammonium chloride with addition of 0.4 wt% amorphous silica

To the prepared solution of chromium (III) chloride hexahydrate salt in cocoalkylmethyl [polyoxyethylene(15)] ammonium chloride ionic liquid as described in Example 1 was added an amorphous silica aqueous colloidal solution which contained 8 wt% of active compound. The concentration of the amorphous silica in the prepared solution, expressed as the quantity of the active compound, was 4 g/kg.

About 250 ml of that solution was poured into the Hull cell described in Example 1. The cell was heated to a temperature of about 80°C.

The same pretreatment of the carbon steel substrate (cathode) as in Example 1 was performed, and again platinized titanium plate was applied as the anode. The potential difference was set to 30 V. The liquid was agitated using a centrally positioned top-entering impeller. The current flow between the electrodes was monitored on a meter connected in series.

After several hours of submission to the current, the cathode was disconnected from the power source and taken out of the cell. The plate was washed in water and acetone and then dried. Chemical analysis by scanning electron microscopy combined with X-ray dispersion (SEM/EDX) of the substrate confirmed deposition of chromium onto the carbon steel plate. The deposited layer thickness, measured using a thickness measurement device (Fischer, Germany) and by cross-cut metallographic analysis, was found to be ranging from 1 to 9 µm.

### Example 4 - Electroplating of chromium from CrCl₃ hexahydrate salt onto carbon steel in coco alkyl methyl [polyoxyethylene(15)] ammonium chloride with addition of 1 wt% of carbon black

To the prepared solution of chromium (III) chloride hexahydrate salt in cocoalkylmethyl [polyoxyethylene(15)] ammonium chloride ionic liquid as described in Example 1 carbon black was added. The concentration of the carbon black in the prepared mixture was 10 g/kg.

About 250 ml of that mixture was poured into the Hull cell described in Example 1. The cell was heated to a temperature of about 70°C.

The same pretreatment of the carbon steel substrate (cathode) as in Example 1 was performed, and again platinized titanium plate was applied as the anode. The potential difference was set to 30 V. The liquid was agitated using a centrally positioned top-entering impeller. The current flow between the electrodes was monitored on a meter connected in series.

After several hours of submission to the current, the cathode was disconnected from the power source and taken out of the cell. The plate was washed in water and acetone and then dried. Chemical analysis by scanning electron microscopy combined with X-ray dispersion (SEM/EDX) of the substrate confirmed deposition of chromium onto the carbon steel plate. The deposited layer thickness, measured using a thickness measurement device (Fischer, Germany), was found to be ranging from 1 to 7 µm. The same thickness values were found by cross-cut metallographic analysis of the substrate samples.

## Claims

1. Use of an additive selected from the group consisting of amorphous silica, graphite powder, and a mixture thereof in a process to electroplate or electropolish a metal on a substrate using an ionic liquid as the electrolyte to increase metal layer thickness.

2. Use of the additive according to claim 1 wherein the ionic liquid is selected from the group consisting of N⁺R₁R₂R₃R₄ X⁻, N⁺R₅R₆R₇R₈ Y⁻, and mixtures thereof, wherein any one of R₁ to R₈ independently represents a hydrogen, alkyl, cycloalkyl, aryl, or aralkyl group that may be substituted with a group selected from OH, Cl, Br, F, I, phenyl, NH₂, CN, NO₂, COOR₉, CHO, COR₉, or OR₉, wherein at least one of R₁ to R₄ is an, optionally branched, fatty alkyl chain, wherein R₂ can be a (C₂-C₆ alkyl)-N⁺R₁₆R₁₇R₁₈ group with R₁₆, R₁₇, R₁₈ being similar to R₁, R₃, R₄, respectively, or a C₁ to C₄ alkyl chain, and wherein one or more of R₁ to R₈ can be a (poly)oxyalkylene group wherein the alkylene is a C₁ to C₄ alkylene and the total number of oxyalkylene units can be from 1 to 50 oxyalkylene units, and wherein at least one of R₁ to R₈ is a C₁ to C₄ alkyl chain, wherein R₉ is an alkyl or cycloalkyl group, wherein X⁻ is an anion compatible with the N⁺R₁R₂R₃R₄ ammonium cation, such as a halogenide anion, a carboxylate anion, a sulphate (both organic and inorganic sulphate), sulphonate, carbonate, nitrate, nitrite, thiocyanate, hydroxide, saccharinate anion, or sulphonylimide anion, and wherein Y⁻ is an anion having a sulfonylimide anion or an N-acyl sulphonylimide anion (-CO-N⁻-SO₂-) functionality.

3. Use of the additive according to claim 1 or 2 wherein the metal which is electroplated or electropolished on the substrate originates from a metal source either being a metal salt selected from the group consisting of chromium, aluminium, titanium, zinc and copper salts, or an anode selected from the group consisting of chromium, aluminium, titanium, zinc, and copper anodes.

4. Use of the additive according to any one of the preceding claims wherein the molar ratio of the cation of the ionic liquid to the metal cation of the metal salt or derived from the metal anode is between 1,000 : 1 and 3 :1, preferably between 100:1 and 7:1.

5. Use of the additive according to claim 4 in an amount of between 0.1 wt% and 5 wt%, based on the total weight of electrolyte.

6. Use of the additive according to any one of the preceding claims wherein the ionic liquid is selected from the group consisting of choline saccharinate, choline acesulphamate, hexadecyltrimethyl ammonium chloride, octadecyltrimethyl ammonium chloride, cocotrimethyl ammonium chloride, tallowtrimethyl ammonium chloride, hydrogenated tallowtrimethyl ammonium chloride, hydrogenated palmtrimethyl ammonium chloride, oleyltrimethyl ammonium chloride, soyatrimethyl ammonium chloride, cocobenzyldimethyl ammonium chloride, C₁₂₋₁₆-alkylbenzyldimethyl ammonium chloride, hydrogenated tallowbenzyldimethyl ammonium chloride, dioctyldimethyl ammonium chloride, didecyldimethyl ammonium chloride, dicocodimethyl ammonium nitrite, dicocodimethyl ammonium chloride, di(hydrogenated tallow)dimethyl ammonium chloride, di(hydrogenated tallow)benzylmethyl ammonium chloride, ditallowdimethyl ammonium chloride, dioctadecyldimethyl ammonium chloride, hydrogenated tallow(2-ethylhexyl)dimethyl ammonium chloride, hydrogenated tallow(2-ethylhexyl)dimethyl ammonium methylsulphate, trihexadecylmethyl ammonium chloride, octadecylmethylbis(2-hydroxyethyl) ammonium chloride, cocobis(2-hydroxyethyl)methyl ammonium nitrate, cocobis(2-hydroxyethyl)methyl ammonium chloride, cocobis(2-hydroxyethyl)benzyl ammonium chloride, oleylbis(2-hydroxyethyl)methyl ammonium chloride, coco[polyoxyethylene(15)]methyl ammonium chloride, coco[polyoxyethylene(15)]methyl ammonium methylsulphate, coco[polyoxyethylene(17)]methyl ammonium chloride, octadecyl[polyoxyethylene(15)]methyl ammonium chloride, hydrogenated tallow[polyoxyethylene(15)]methyl ammonium chloride, tris(2-hydroxyethyl)tallow ammonium acetate, tallow-1,3-propane pentamethyl diammonium dichloride.

7. A method to electroplate or electropolish a metal on a metal substrate wherein an ionic liquid is selected from the group consisting of N⁺R₁R₂R₃R₄ X⁻, N⁺R₅R₆R₇R₈ Y⁻, and mixtures thereof, wherein any one of R₁ to R₈ independently represents a hydrogen, alkyl, cycloalkyl, aryl, or aralkyl group that may be substituted with a group selected from OH, Cl, Br, F, I, phenyl, NH₂, CN, NO₂, COOR₉, CHO, COR₉, or OR₉, wherein at least one of R₁ to R₄ is an, optionally branched, fatty alkyl chain, wherein R₂ can be a (C₂-C₆ alkyl)-N⁺R₁₆R₁₇R₁₈ group with R₁₆, R₁₇, R₁₈ being similar to R₁, R₃, R₄, respectively, or a C₁ to C₄ alkyl chain, and wherein one or more of R₁ to R₈ can be a (poly)oxyalkylene group wherein the alkylene is a C₁ to C₄ alkylene and the total number of oxyalkylene units can be from 1 to 50 oxyalkylene units, and wherein at least one of R₁ to R₈ is a C₁ to C₄ alkyl chain, wherein R₉ is an alkyl or cycloalkyl group, wherein X- is an anion compatible with the N⁺R₁R₂R₃R₄ ammonium cation, such as a halogenide anion, a carboxylate anion, a sulphate (both organic and inorganic sulphate), sulphonate, carbonate, nitrate, nitrite, thiocyanate, hydroxide, saccharinate anion, or sulphonylimide anion, and wherein Y⁻ is an anion having a sulfonylimide anion or an N-acyl sulphonylimide anion (-CO-N⁻-SO₂-) functionality; wherein a metal salt added to said ionic liquid or a metal anode is employed as metal source; and wherein said ionic liquid comprises at least 0.01 wt%, based on the total weight of electrolyte, of an additive selected from the group consisting of amorphous silica, graphite powder, and of a mixture thereof.

8. A method according to claim 7 wherein the metal which is electroplated or electropolished on the substrate originates from a metal source either being a metal salt selected from the group consisting of chromium, aluminium, titanium, zinc and copper salts, or an anode selected from the group consisting of chromium, aluminium, titanium, zinc, and copper anodes.

9. A method according to claim 7 or 8 wherein the molar ratio of the cation of the ionic liquid to the metal cation of the metal salt or derived from the metal anode is between 1,000 : 1 and 3 :1, and preferably between 100:1 and 7:1.

10. A method according to any one of claims 7-9 wherein the ionic liquid is selected from the group consisting of choline saccharinate, choline acesulphamate, hexadecyltrimethyl ammonium chloride, octadecyltrimethyl ammonium chloride, cocotrimethyl ammonium chloride, tallowtrimethyl ammonium chloride, hydrogenated tallowtrimethyl ammonium chloride, hydrogenated palmtrimethyl ammonium chloride, oleyltrimethyl ammonium chloride, soyatrimethyl ammonium chloride, cocobenzyldimethyl ammonium chloride, C₁₂₋₁₆-alkylbenzyldimethyl ammonium chloride, hydrogenated tallowbenzyldimethyl ammonium chloride, dioctyldimethyl ammonium chloride, didecyldimethyl ammonium chloride, dicocodimethyl ammonium nitrite, dicocodimethyl ammonium chloride, di(hydrogenated tallow)dimethyl ammonium chloride, di(hydrogenated tallow)benzylmethyl ammonium chloride, ditallowdimethyl ammonium chloride, dioctadecyldimethyl ammonium chloride, hydrogenated tallow(2-ethylhexyl)dimethyl ammonium chloride, hydrogenated tallow(2-ethylhexyl)dimethyl ammonium methylsulphate, trihexadecylmethyl ammonium chloride, octadecylmethylbis(2-hydroxyethyl) ammonium chloride, cocobis(2-hydroxyethyl)methyl ammonium nitrate, cocobis(2-hydroxyethyl)methyl ammonium chloride, cocobis(2-hydroxyethyl)benzyl ammonium chloride, oleylbis(2-hydroxyethyl)methyl ammonium chloride, coco[polyoxyethylene(15)]methyl ammonium chloride, coco[polyoxyethylene(15)]methyl ammonium methylsulphate, coco[polyoxyethylene(17)]methyl ammonium chloride, octadecyl[polyoxyethylene(15)]methyl ammonium chloride, hydrogenated tallow[polyoxyethylene(15)]methyl ammonium chloride, tris(2-hydroxyethyl)tallow ammonium acetate, tallow-1,3-propane pentamethyl diammonium dichloride.

## Patentansprüche

1. Verwendung eines Additivs ausgewählt aus der Gruppe bestehend aus amorphem Siliziumdioxid, Graphitpulver und einem Gemisch davon bei einem Elektroplating-Verfahren oder einem Verfahren zum elektrolytischen Polieren eines Metalls auf einem Substrat unter Verwendung einer ionischen Flüssigkeit als Elektrolyt, um die Dicke der Metallschicht zu erhöhen.

2. Verwendung des Additivs gemäß Anspruch 1, wobei die ionische Flüssigkeit ausgewählt ist aus der Gruppe bestehend aus N⁺R₁R₂R₃R₄X⁻, N⁺R₅R₆R₇R₈Y⁻ und Gemischen davon, wobei jeder der Rest R₁ bis R₈ unabhängig einen Wasserstoff-, Alkyl-, Cycloalkyl-, Aryl- oder Aralkylrest darstellt, welcher mit einem Rest, ausgewählt aus OH, Cl, Br, F, I, Phenyl, NH₂, CN, NO₂, COOR₉, CHO, COR₉ oder OR₉ substituiert sein kann, wobei mindestens einer der Reste R₁ bis R₄ eine, gegebenenfalls verzweigte, Fettalkylkette ist, wobei R₂ ein (C₂-C₆-Alkyl)-N⁺R₁₆R₁₇R₁₈-Rest sein kann, wobei R₁₆, R₁₇, R₁₈ jeweils ähnlich wie R₁, R₃ oder R₄ sind, oder eine C₁- bis C₄-Alkylkette ist und wobei einer oder mehrere der Reste R₁ bis R₈ eine (Poly)oxyalkylengruppe sein kann, wobei das Alkylen ein C₁- bis C₄-Alkylen ist und die Gesamtzahl der Oxyalkyleneinheiten 1 bis 50 Oxyalkyleneinheiten betragen kann, und wobei mindestens einer der Reste R₁ bis R₈ eine C₁₋ bis C₄-Alkylkette ist, wobei R₉ ein Alkyl- oder Cycloalkylrest ist, wobei X⁻ ein Anion darstellt, welches mit dem N⁺R₁R₂R₃R₄-Ammoniumkation kompatibel ist, wie ein Halogenidanion, ein Carboxylatanion, ein Sulphat (sowohl organisches also auch anorganisches Sulphat), Sulphonat, Carbonat, Nitrat, Nitrit, Thiocyanat, Hydroxid, Saccharinatanion oder Sulfonylimidanion und wobei Y⁻ ein Anion ist, welches eine Sulfonylimidanion- oder eine N-Acylsulfonylimidanion-(-CO-N⁻-SO₂-)-Funktionalität aufweist.

3. Verwendung des Additivs gemäß Anspruch 1 oder 2, wobei das Metall, welches auf dem Substrat dem Elektroplating unterzogen oder elektrolytisch poliert wird, aus einer Metallquelle stammt, die entweder ein Metallsalz, ausgewählt aus der Gruppe bestehend aus Chrom-, Aluminium-, Titan-, Zink- und Kupfersalzen, oder eine Anode, ausgewählt aus der Gruppe bestehend aus Chrom-, Aluminium-, Titan-, Zink- und Kupferanoden, ist.

4. Verwendung des Additivs gemäß einem der vorhergehenden Ansprüche, wobei das Molverhältnis des Kations der ionischen Flüssigkeit zu dem Metallkation des Metallsalzes oder dem Metallkation, welches aus der Metallanode stammt, zwischen 1,000 : 1 und 3 : 1, vorzugsweise zwischen 100 : 7 und 7 : 1 liegt.

5. Verwendung des Additivs gemäß Anspruch 4 in einer Menge zwischen 0,1 Gew.-% und 5 Gew.-%, bezogen auf das Gesamtgewicht des Elektrolyts.

6. Verwendung des Additivs gemäß einem der vorhergehenden Ansprüche, wobei die ionische Flüssigkeit ausgewählt ist aus der Gruppe bestehend aus Cholinsaccharinat, Cholinacesulphamat, Hexadecyltrimethylammoniumchlorid, Octadecyltrimethylammoniumchlorid, Cocotrimethylammoniumchlorid, Talgtrimethylammoniumchlorid, hydriertem Talgtrimethylammoniumchlorid, hydriertem Palmtrimethylammoniumchlorid, Oleyltrimethylammoniumchlorid, Soyatrimethylammoniumchlorid, Cocobenzyldimethylammoniumchlorid, C₁₂₋₁₆-Alkylbenzyldimethylammoniumchlorid, hydriertem Talgbenzyldimethylammoniumchlorid, Dioctyldimethylammoniumchlorid, Didecyldimethylammoniumchlorid, Dicocodimethylammoniumnitrit, Dicocodimethylammoniumchlorid, Di(hydriertem Talg)dimethylammoniumchlorid, Di(hydriertem Talg)benzylmethylammoniumchlorid, Ditalgdimethylammoniumchlorid, Dioctadecyldimethylammoniumchlorid, hydriertem Talg(2-ethylhexyl)dimethylammoniumchlorid, hydriertem Talg(2-ethylhexyl)dimethylammoniummethylsulphat, Trihexadecylmethylammoniumchlorid, Octadecylmethylbis(2-hydroxyethyl)ammoniumchlorid, Cocobis(2-hydroxyethyl)methylammoniumnitrat, Cocobis(2-hydroxyethyl)methylammoniumchlorid, Cocobis(2-hydroxyethyl)benzylammoniumchlorid, Oleylbis(2-hydroxyethyl)methylammoniumchlorid, Coco[polyoxyethylen(15)]methylammoniumchlorid, Coco[polyoxyethylen(15)]methylammoniummethylsulphat, Coco[polyoxyethylen(17)]methylammoniumchlorid, Octadecyl[polyoxyethylen(15)]methylammoniumchlorid, hydriertem Talg[polyoxyethylen(15)]methylammoniumchlorid, tris(2-Hydroxyethyl)talgammoniumacetat, Talg-1,3-propanpentamethyldiammoniumdichlorid.

7. Ein Verfahren zum Elektroplating oder zum elektrolytischen Polieren eines Metalls auf einem Metallsubstrat, wobei eine ionische Flüssigkeit ausgewählt ist aus der Gruppe bestehend aus N⁺R₁R₂R₃R₄X⁻, N⁺R₅R₆R₇R₈Y⁻ und Gemischen davon, wobei jeder der Reste R₁ bis R₈ unabhängig einen Wasserstoff-, Alkyl-, Cycloalkyl-, Aryl- oder Aralkylrest darstellt, welcher mit einem Rest ausgewählt aus OH, Cl, Br, F, I, Phenyl, NH₂, CN, NO₂, COOR₉, CHO, COR₉ oder OR₉ substituiert sein kann, wobei mindestens einer der Reste R₁ bis R₄ eine, gegebenenfalls verzweigte, Fettalkylkette ist, wobei R₂ ein (C₂-C₆-Alkyl)-N⁺R₁₆R₁₇R₁₈-Rest sein kann, wobei R₁₆, R₁₇, R₁₈ jeweils ähnlich wie R₁, R₃ oder R₄ sind, oder eine C₁- bis C₄-Alkylkette ist und wobei einer oder mehrere der Reste R₁ bis R₈ eine (Poly)oxyalkylengruppe sein kann, wobei das Alkylen ein C₁- bis C₄-Alkylen ist und die Gesamtzahl der Oxyalkyleneinheiten 1 bis 50 Oxyalkyleneinheiten betragen kann, und wobei mindestens einer der Reste R₁ bis R₈ eine C₁₋ bis C₄-Alkylkette ist, wobei R₉ ein Alkyl- oder Cycloalkylrest ist, wobei X⁻ ein Anion darstellt, welches mit dem N⁺R₁R₂R₃R₄-Ammoniumkation kompatibel ist, wie ein Halogenidanion, ein Carboxylatanion, ein Sulphat (sowohl organisches also auch anorganisches Sulphat), Sulphonat, Carbonat, Nitrat, Nitrit, Thiocyanat, Hydroxid, Saccharinatanion oder Sulfonylimidanion und wobei Y⁻ ein Anion ist, welches eine Sulfonylimidanion- oder eine N-Acylsulfonylimidanion(-CO-N⁻-SO₂-)-Funktionalität aufweist; wobei ein zur ionischen Flüssigkeit zugegebenes Metallsalz oder eine Metallanode als Metallquelle verwendet wird; und wobei die ionische Flüssigkeit mindestens 0,01 Gew.-% eines Additivs, ausgewählt aus der Gruppe bestehend aus amorphem Siliziumdioxid, Graphitpulver und einem Gemisch davon, umfasst, bezogen auf das Gesamtgewicht des Elektrolyts.

8. Ein Verfahren gemäß Anspruch 7, wobei das Metall, welches auf dem Substrat dem Elektroplating unterzogen oder elektrolytisch poliert wird, aus einer Metallquelle stammt, welche entweder ein Metallsalz, ausgewählt aus der Gruppe bestehend aus Chrom-, Aluminium-, Titan-, Zink- und Kupfersalzen oder eine Anode, ausgewählt aus der Gruppe bestehend aus Chrom-, Aluminium-, Titan-, Zink- und Kupferanoden, ist.

9. Ein Verfahren gemäß Anspruch 7 oder 8, wobei das Molverhältnis des Kations der ionischen Flüssigkeit zu dem Metallkation des Metallsalzes oder dem Metallkation, welches aus der Metallanode stammt, zwischen 1,000 : 1 und 3 : 1, und vorzugweise zwischen 100 : 1 und 7 : 1 liegt.

10. Ein Verfahren gemäß einem der Ansprüche 7-9, wobei die ionische Flüssigkeit ausgewählt ist aus der Gruppe bestehend aus Cholinsaccharinat, Cholinacesulphamat, Hexadecyltrimethylammoniumchlorid, Octadecyltrimethylammoniumchlorid, Cocotrimethylammoniumchlorid, Talgtrimethylammoniumchlorid, hydriertem Talgtrimethylammoniumchlorid, hydriertem Palmtrimethylammoniumchlorid, Oleyltrimethylammoniumchlorid, Soyatrimethylammoniumchlorid, Cocobenzyldimethylammoniumchlorid, C₁₂₋₁₆-Alkylbenzyldimethylammoniumchlorid, hydriertem Talgbenzyldimethylammoniumchlorid, Dioctyldimethylammoniumchlorid, Didecyldimethylammoniumchlorid, Dicocodimethylammoniumnitrit, Dicocodimethylammoniumchlorid, Di(hydriertem Talg)dimethylammoniumchlorid, Di(hydriertem Talg)benzylmethylammoniumchlorid, Ditalgdimethylammoniumchlorid, Dioctadecyldimethylammoniumchlorid, hydriertem Talg(2-ethylhexyl)dimethylammoniumchlorid, hydriertem Talg(2-ethylhexyl)dimethylammoniummethylsulphat, Trihexadecylmethylammoniumchlorid, Octadecylmethylbis(2-hydroxyethyl)ammoniumchlorid, Cocobis(2-hydroxyethyl)methylammoniumnitrat, Cocobis(2-hydroxyethyl)methylammoniumchlorid, Cocobis(2-hydroxyethyl)benzylammoniumchlorid, Oleylbis(2-hydroxyethyl)methylammoniumchlorid, Coco[polyoxyethylen(15)]methylammoniumchlorid, Coco[polyoxyethylen(15)]methylammoniummethylsulphat, Coco[polyoxyethylen(17)]methylammoniumchlorid, Octadecyl[polyoxyethylen(15)]methylammoniumchlorid, hydriertem Talg[polyoxyethylen(15)]methylammoniumchlorid, tris(2-Hydroxyethyl)talgammoniumacetat, Talg-1,3-propanpentamethyldiammoniumdichlorid.

## Revendications

1. Utilisation d'un additif choisi dans le groupe constitué par la silice amorphe, la poudre de graphite, et un de leurs mélanges, dans un procédé de placage électrolytique ou de polissage électrolytique d'un métal sur un substrat utilisant un liquide ionique en tant qu'électrolyte pour augmenter l'épaisseur de la couche de métal.

2. Utilisation de l'additif selon la revendication 1, dans laquelle le liquide ionique est choisi dans le groupe constitué par N⁺R₁R₂R₃R₄X⁻, N⁺R₅R₆R₇R₈Y⁻, et leurs mélanges, où l'un quelconque de R₁ à R₈ représente indépendamment un hydrogène ou un groupe alkyle, cycloalkyle, aryle ou aralkyle qui peut être substitué par un groupe choisi parmi OH, Cl, Br, F, I, phényle, NH₂, CN, NO₂, COOR₉, CHO, COR₉ et OR₉, où au moins l'un de R₁ à R₄ est une chaîne alkyle gras éventuellement ramifiée, où R₂ peut être un groupe (alkyl en C₂ à C₆)-N⁺R₁₆R₁₇R₁₈, R₁₆, R₁₇ et R₁₈ étant respectivement similaires à R₁, R₃ et R₄, ou une chaîne alkyle en C₁ à C₄, et où un ou plusieurs de R₁ à R₈ peut être un groupe (poly)oxyalkylène dans lequel l'alkylène est un alkylène en C₁ à C₄ et le nombre total de motifs oxyalkylène peut être de 1 à 50 motifs oxyalkylène, et où au moins l'un de R₁ à R₈ est une chaîne alkyle en C₁ à C₄, où R₉ est un groupe alkyle ou cycloalkyle, où X⁻ est un anion compatible avec le cation ammonium N⁺R₁R₂R₃R₄, tel qu'un anion halogénure, un anion carboxylate, un anion sulfate (sulfate tant organique qu'inorganique), sulfonate, carbonate, nitrate, nitrite, thiocyanate, hydroxyde, saccharinate, ou un anion sulfonylimide, et où Y⁻ est un anion ayant une fonctionnalité d'anion sulfonylimide ou d'anion N-acylsulfonylimide (-CO-N⁻-SO₂-).

3. Utilisation de l'additif selon la revendication 1 ou 2, dans laquelle le métal qui est soumis à un placage électrolytique ou à un polissage électrolytique sur le substrat provient d'une source de métal qui est soit un sel métallique choisi dans le groupe constitué par les sels de chrome, aluminium, titane, zinc et cuivre, soit une anode choisie dans le groupe constitué par les anodes en chrome, aluminium, titane, zinc et cuivre.

4. Utilisation de l'additif selon l'une quelconque des revendications précédentes, dans laquelle le rapport molaire du cation du liquide ionique au cation métallique du sel métallique ou dérivant de l'anode métallique est compris entre 1000/1 et 3/1, de préférence entre 100/1 et 7/1.

5. Utilisation de l'additif selon la revendication 4 en une quantité comprise entre 0,1 % en poids et 5 % en poids par rapport au poids total de l'électrolyte.

6. Utilisation de l'additif selon l'une quelconque des revendications précédentes, dans laquelle le liquide ionique est choisi dans le groupe constitué par le saccharinate de choline, l'acésulfamate de choline, le chlorure d'hexadécyltriméthylammonium, le chlorure d'octadécyltriméthylammonium, le chlorure de (coprah) triméthylammonium, le chlorure de (suif-) triméthylammonium, le chlorure de (suif- hydrogéné) triméthylammonium, le chlorure de (palmityl hydrogéné) triméthylammonium, le chlorure d'oléyltriméthylammonium, le chlorure de (soja-) triméthylammonium, le chlorure de (coprah) benzyldiméthylammonium, le chlorure de (alkyl en C₁₂ à C₁₆) benzyldiméthylammonium, le chlorure de (suif hydrogéné) benzyldiméthylammonium, le chlorure de dioctyldiméthylammonium, le chlorure de didécyldiméthylammonium, le nitrite de di(coprah) diméthylammonium, le chlorure de di(coprah) diméthylammonium, le chlorure de di(suif hydrogéné) diméthylammonium, le chlorure de di(suif hydrogéné) benzylméthylammonium, le chlorure de di(suif) diméthylammonium, le chlorure de dioctadécyldiméthylammonium, le chlorure de (suif hydrogéné)-(2-éthylhexyl) diméthylammonium, le méthylsulfate de (suif hydrogéné)-(2-éthylhexyl) diméthylammonium, le chlorure de trihexadécylméthylammonium, le chlorure d'octadécylméthyl-bis(2-hydroxyéthyl) ammonium, le nitrate de (coprah)bis(2-hydroxyéthyl) méthylammonium, le chlorure de (coprah)bis(2-hydroxyéthyl) méthylammonium, le chlorure d e (coprah)bis(2-hydroxyéthyl) benzylammonium, le chlorure d'oléylbis(2-hydroxyéthyl) méthylammonium, le chlorure de (coprah) méthylammonium polyoxyéthyléné(15), le méthylsulfate de (coprah) méthylammonium polyoxy-éthyléné(15), le chlorure de (coprah) méthylammonium polyoxyéthyléné(17), le chlorure d'octadécylméthylammonium polyoxyéthyléné(15), le chlorure de (suif hydrogéné) méthylammonium polyoxyéthyléné(15), l'acétate de tris(2-hydroxyéthyl)-(suif) ammonium, le dichlorure de (suif)-1,3-propanepentaméthyldiammonium.

7. Procédé de placage électrolytique ou de polissage électrolytique d'un métal sur un substrat métallique, dans lequel un liquide ionique est choisi dans le groupe constitué par N⁺R₁R₂R₃R₄X⁻, N⁺R₅R₆R₇R₈Y⁻, et leurs mélanges, où l'un quelconque de R₁ à R₈ représente indépendamment un hydrogène ou un groupe alkyle, cycloalkyle, aryle ou aralkyle qui peut être substitué par un groupe choisi parmi OH, Cl, Br, F, I, phényle, NH₂, CN, NO₂, COOR₉, CHO, COR₉ et OR₉, où au moins l'un de R₁ à R₄ est une chaîne alkyle gras éventuellement ramifiée, où R₂ peut être un groupe (alkyl en C₂ à C₆)-N⁺R₁₆R₁₇R₁₈, R₁₆, R₁₇ et R₁₈ étant respectivement similaires à R₁, R₃ et R₄, ou une chaîne alkyle en C₁ à C₄, et où un ou plusieurs de R₁ à R₈ peut être un groupe (poly)oxyalkylène dans lequel l'alkylène est un alkylène en C₁ à C₄ et le nombre total de motifs oxyalkylène peut être de 1 à 50 motifs oxyalkylène, et où au moins l'un de R₁ à R₈ est une chaîne alkyle en C₁ à C₄, où R₉ est un groupe alkyle ou cycloalkyle, où X⁻ est un anion compatible avec le cation ammonium N⁺R₁R₂R₃R₄, tel qu'un anion halogénure, un anion carboxylate, un anion sulfate (sulfate tant organique qu'inorganique), sulfonate, carbonate, nitrate, nitrite, thiocyanate, hydroxyde, saccharinate, ou un anion sulfonylimide, et où Y⁻ est un anion ayant une fonctionnalité d'anion sulfonylimide ou d'anion N-acylsulfonylimide (-CO-N⁻-SO₂-) ; dans lequel un sel métallique ajouté audit liquide ionique ou une anode métallique est employé en tant que source de métal ; et dans lequel ledit liquide ionique comprend au moins 0,01 % en poids, par rapport au poids total de l'électrolyte, d'un additif choisi dans le groupe constitué par la silice amorphe, la poudre de graphite, et un de leurs mélanges.

8. Procédé selon la revendication 7, dans lequel le métal qui a été soumis à un placage électrolytique ou à un polissage électrolytique sur le substrat provient d'une source de métal qui est soit un sel métallique choisi dans le groupe constitué par les sels de chrome, aluminium, titane, zinc et cuivre, soit une anode choisie dans le groupe constitué par les anodes en chrome, aluminium, titane, zinc et cuivre.

9. Procédé selon la revendication 7 ou 8, dans lequel le rapport molaire du cation du liquide ionique au cation métallique du sel métallique ou dérivant de l'anode métallique est compris entre 1000/1 et 3/1, de préférence entre 100/1 et 7/1.

10. Procédé selon l'une quelconque des revendications 7 à 9, dans lequel le liquide ionique est choisi dans le groupe constitué par le saccharinate de choline, l'acésulfamate de choline, le chlorure d'hexadécyltriméthylammonium, le chlorure d'octadécyltriméthylammonium, le chlorure de (coprah) triméthylammonium, le chlorure de suiftriméthylammonium, le chlorure de (suif hydrogéné) triméthylammonium, le chlorure de (palmityl hydrogéné) triméthylammonium, le chlorure d'oléyltriméthylammonium, le chlorure de (soja) triméthylammonium, le chlorure de (coprah) benzyldiméthylammonium, le chlorure de (alkyl en C₁₂ à C₁₆) benzyldiméthylammonium, le chlorure de (suif hydrogéné) benzyldiméthylammonium, le chlorure de dioctyldiméthylammonium, le chlorure de didécyldiméthylammonium, le nitrite de di(coprah) diméthylammonium, le chlorure de di(coprah) diméthylammonium, le chlorure de di(suif hydrogéné) diméthylammonium, le chlorure de di(suif hydrogéné) benzylméthylammonium, le chlorure de di(suif) diméthylammonium, le chlorure de dioctadécyldiméthylammonium, le chlorure de (suif hydrogéné)-(2-éthylhexyl) diméthylammonium, le méthylsulfate de (suif hydrogéné)-(2-éthylhexyl) diméthylammonium, le chlorure de trihexadécylméthylammonium, le chlorure d'octadécylméthyl-bis(2-hydroxyéthyl) ammonium, le nitrate de (coprah)-bis(2-hydroxyéthyl) méthylammonium, le chlorure de (coprah)bis(2-hydroxyéthyl)méthylammonium, le chlorure de (coprah)bis(2-hydroxyéthyl) benzylammonium, le chlorure d'oléylbis(2-hydroxyéthyl) méthylammonium, le chlorure de (coprah) méthylammonium polyoxyéthyléné(15), le méthyl-sulfate de (coprah) méthylammonium polyoxyéthyléné(15), le chlorure de (coprah) méthylammonium polyoxy-éthyléné(17), le chlorure d'octadécylméthylammonium polyoxyéthyléné(15), le chlorure de (suif hydrogéné) méthylammonium polyoxyéthyléné(15), l'acétate de tris(2-hydroxyéthyl)-(suif) ammonium, le dichlorure de (suif)-1,3-propanepentaméthyldiammonium.
